

## UNITED STATES PATENT OFFICE

2,355,219

## HYDROGENATION OF ARYL CARBOXYLIC ACIDS

Vladimir N. Ipatieff and Vladimir Haensel, Riverside, Ill., assignors to Universal Oil Products Company, Chicago, Ill., a corporation of Delaware

No Drawing. Application May 31, 1943,  
Serial No. 489,153

10 Claims. (Cl. 260—668)

This invention relates to the use of particular catalytic materials in reactions involving hydrogenation of aryl carboxylic acids.

An object of this invention is the hydrogenation of aromatic carboxylic acids so as to produce therefrom aromatic hydrocarbons or alkylated aromatic hydrocarbons having the same number of carbon atoms per molecule as present in said aromatic carboxylic acids.

Another object of this invention is the hydrogenation of an aromatic carboxylic acid in the presence of a catalyst produced by subjecting to reduction a composite formed from copper oxide and at least another oxide selected from the group consisting of aluminum oxide and zinc oxide whereby to convert the carboxylic acid group into a methyl group with substantially no other influence on the aromatic carboxylic acid.

A further object of this invention is the production of an aromatic hydrocarbon by the hydrogenation of an aromatic monocarboxylic acid in the presence of a catalyst comprising essentially a composite of reduced copper and at least one of the oxides selected from the group consisting of aluminum oxide and zinc oxide.

A still further object of this invention is the hydrogenation of a member selected from the group consisting of aryl carboxylic acids and anhydrides of aryl carboxylic acids to produce alkyl aryl compounds including alkyl aromatic hydrocarbons, alkyl aryl carbinols, aromatic esters, and aromatic carbonyl compounds such as aromatic aldehydes.

In one specific embodiment the present invention comprises a process for producing alkylated aromatic hydrocarbons by reacting an aryl carboxylic acid and hydrogen in the presence of a catalyst comprising essentially a composite of reduced copper and at least one of the oxides selected from the group consisting of aluminum oxide and zinc oxide.

Aryl carboxylic acids which are utilizable as starting materials in the present process may be obtained from any source and may comprise monocyclic and polycyclic aromatic carboxylic acids including both the monobasic and also polybasic acids. Aromatic carboxylic acids which may be hydrogenated as herein set forth also include compounds in which one or more of the hydrogen atoms of an aromatic ring may be considered to be replaced by an organic acid group generally referred to as a carboxyl group. Aromatic carboxylic acids also include the aryl fatty acids such as phenyl acetic acid, the different isomeric phenyl propionic acids, etc. in which one of the hydrogen atoms of the alkyl group of an aliphatic carboxylic acid may be considered to be replaced by a phenyl group or other aromatic hydrocarbon group.

For purposes of reference some of the aromatic

carboxylic acids are listed in the following table together with their melting points and in a few instances their boiling points where the latter values are available.

| Some aryl carboxylic acids |                                      |               |               |
|----------------------------|--------------------------------------|---------------|---------------|
|                            | Aromatic acids                       | Melting point | Boiling point |
| 10                         | <i>Mono-carboxylic</i>               | °C.           | °C.           |
|                            | Benzoin                              | 120           | 250           |
|                            | o-Toluic                             | 102           |               |
|                            | m-Toluic                             | 110           | 263           |
|                            | p-Toluic                             | 188           | 275           |
|                            | o-Ethylbenzoic                       | 68            |               |
|                            | m-Ethylbenzoic                       | 47            |               |
|                            | p-Ethylbenzoic                       | 112           |               |
| 15                         | 1,2-dimethyl-3-benzoic               | 144           |               |
|                            | 1,3-dimethyl-2-benzoic               | 98            |               |
|                            | 1,4-dimethyl-2-benzoic               | 132           | 268           |
|                            | o-n-Propyl benzoic                   | 58            |               |
|                            | p-n-Propyl benzoic                   | 138           |               |
|                            | o-iso-Propyl benzoic                 | 51            |               |
|                            | p-iso-Propyl benzoic                 | 117           |               |
| 20                         | 1,2,3-trimethyl-4-benzoic            | 167           |               |
|                            | 1,2,4-trimethyl-5-benzoic            | 150           |               |
|                            | 1,3,5-mesitylene carboxylic          | 152           |               |
|                            | 1,2,3,4-tetramethyl-5-benzoic        | 165           |               |
|                            | Pentamethylbenzoic                   | 210           |               |
| 25                         | <i>Phenyl-fatty acids</i>            |               |               |
|                            | Phenyl acetic                        | 76            | 262           |
|                            | β-Phenyl propionic                   | 47            | 280           |
|                            | α-Phenyl propionic                   | 78            | 262           |
|                            | α-Phenyl-iso-butyric                 | 78            | 150 at 10 mm. |
|                            | β-Phenyl-butyric                     | 39            |               |
|                            | α-Phenyl-butyric                     | 52            |               |
| 30                         | <i>Acids of polycyclic aromatics</i> |               |               |
|                            | α-Naphthoic                          | 160           |               |
|                            | α-Naphthoic                          | 182           |               |
|                            | β-Naphthyl Acetic                    | 131           |               |
|                            | β-Anthracene carboxylic              | 245           |               |
|                            | α-Anthracene carboxylic              | 281           |               |
| 35                         | <i>Aromatic dicarboxylic acids</i>   |               |               |
|                            | Phthalic                             | 213           |               |
|                            | Isophthalic                          | Above 300     |               |
|                            | Terephthalic                         | Sublimes      |               |
|                            | Naphthalic                           | Dec.          |               |
| 40                         |                                      |               |               |
| 45                         |                                      |               |               |
| 50                         |                                      |               |               |
| 55                         |                                      |               |               |

The process of the present invention is also applicable to the hydrogenation of anhydrides of aryl carboxylic acids. The products obtainable by such hydrogenation treatment of these acid anhydrides are essentially the same as those produced by hydrogenation of the corresponding aryl carboxylic acid.

Composites of the above-indicated materials utilizable as catalysts in the hydrogenation of aryl carboxylic acids and their anhydrides may be made by precipitating the carbonates of zinc and copper from aqueous solutions of the metallic salts, particularly the nitrates, by the addition of water soluble carbonates, particularly ammonium carbonate, at ordinary or elevated temperatures. Aluminum hydroxide may be precipitated similarly either in the presence or absence of the carbonates of copper and zinc. The precipitated material so obtained is filtered, carefully washed with water to remove water soluble

salts, dried, and in some cases later formed into particles or pellets of different sizes and shapes. The dried catalyst either in the form of powder, particles, or pellets is then heated in a stream of hydrogen or of a gas mixture containing hydrogen in order to decompose the metal carbonate and to reduce a substantial proportion of the resulting copper oxide to metallic copper in a form having relatively high hydrogenating activity. The metal carbonate may also be decomposed by heating in air prior to being heated in hydrogen to effect reduction.

The composite catalytic material may also be prepared by coprecipitating copper carbonate, zinc carbonate, and/or aluminum hydroxide; or for the preparation of a copper oxide-zinc oxide-aluminum oxide mixture, the zinc carbonate may be first precipitated on alumina followed by precipitation of the basic copper carbonate on the mixture. The proportions of the various components may be varied considerably. A good catalyst is prepared containing 25 parts by weight of zinc, 25 parts by weight of copper, and 50 parts by weight of alumina; while others consist of approximately equal parts by weight of zinc, copper, and alumina. Similarly, composites of copper and alumina also yield highly active catalysts which after reduction with a hydrogen-containing gas comprise essentially copper and alumina, said composites containing from about 1 to about 50% by weight of alumina mixed with reduced copper.

The catalyst granules or pellets of the type hereinabove described may be used as filling materials in suitable heated reactors through which the aryl carboxylic acid and hydrogen are passed at a temperature of from about 200° to about 350° C. and under a pressure of from about 25 to about 300 atmospheres. Under some circumstances it may be advantageous to commingle the aryl carboxylic acid with a solvent such as ethyl alcohol, dioxane, etc. before it is subjected to hydrogenation in the presence of the catalyst. However, when an alcohol is present in the reaction mixture, some of the carboxylic acid may react therewith to form an ester. As the conditions of operation are not necessarily the same for the hydrogenation of the different aryl carboxylic acids, the catalyst temperature, charging rate of said carboxylic acid, and ratio of hydrogen to carboxylic acid employed are chosen to give a high degree of conversion to alkylated aromatic hydrocarbons with a relatively small amount of accompanying decomposition and with substantially no hydrogenation of the aromatic ring of the carboxylic acid to a naphthenic ring.

Alternatively, powdered catalyst of the types herein described may be suspended in the aryl carboxylic acid and the resultant mixture and hydrogen may be passed through a suitable reactor to effect hydrogenation of a substantial proportion of said aryl carboxylic acid. The powdered catalyst may thus be used in the form of a slurry, or it may be mixed with the hydrogen in a so-called fluidized type of operation; and thereafter the hydrogen-catalyst mixture may be contacted with pre-heated aryl carboxylic acid. After such a hydrogenation treatment in the presence of a powdered catalyst the reaction products are separated from the catalyst and fractionated to recover the desired products and to separate unconverted aryl carboxylic acid and used catalyst which are recycled to the reaction zone for further use. A powdered catalyst may thus be used

in either batch or continuous hydrogenation of an aryl carboxylic acid.

The process of this invention is particularly advantageous for producing aromatic hydrocarbons from aryl carboxylic acids since the composite catalyst containing copper and at least one of the oxides selected from the group consisting of aluminum oxide and zinc oxide is able to catalyze the hydrogenation of the carboxylic acid group to a methyl group without simultaneous hydrogenation of the aromatic ring or aromatic rings to naphthenic or cyclohexane rings. A number of catalysts of the prior art have been utilized in hydrogenations of aryl carboxylic acids, but with these catalysts the aromatic ring underwent reduction to a cycloparaffin ring which is generally referred to as a naphthene ring. The catalysts of the present process, however, are sufficiently active to catalyze the conversion of the carboxyl group or carboxyl groups, in case a polycarboxylic acid is being hydrogenated, substantially without affecting the aromatic nucleus of the aryl carboxylic acid.

Hydrogenation catalysts prepared by the process herein set forth which includes precipitating copper carbonate, aluminum hydroxide and/or zinc carbonate, followed by filtering, washing, drying, and reducing as herein set forth, are generally hard and resistant to breakage, have relatively high activities, and do not undergo excessive carbonization during use in hydrogenation of aromatic acids. When carbonization occurs, as after a long period of service, it is usually advisable to burn the carbonaceous deposit from the catalyst by treatment with a gas of controlled oxygen concentration followed by heating in a reducing gas such as hydrogen, carbon monoxide, a mixture of hydrogen and carbon monoxide, or a gas mixture containing a substantial amount of a reducing gas.

The following examples are given to indicate results obtained by the process although these data are not introduced with the intention of unduly limiting the generally broad scope of the invention.

#### Example I

In preparing a copper-alumina catalyst 1442 grams of cupric nitrate trihydrate and 184 grams of aluminum nitrate nonahydrate were dissolved in 12 liters of water. Another solution was prepared by dissolving 770 grams of ammonium carbonate monohydrate in 5 liters of water. Then the ammonium carbonate solution was added slowly with stirring to the solution containing copper nitrate and aluminum nitrate. Upon completion of the precipitation the entire reaction mixture containing precipitated copper carbonate and aluminum hydroxide was heated at 70 to 80° C. during a period of between 0.5 and 1 hour. Upon reaching 80° C. the heating was discontinued and the precipitate was allowed to cool and settle. Then approximately 12 liters of solution were decanted from the precipitate which was then washed by the addition of 12 liters of distilled water. This procedure of washing by decantation was repeated four times and finally the precipitate was separated from the wash water by filtration with suction. The filter cake so obtained was washed again with 2 liters of water and separated by filtration. The washed catalyst was then dried at 240° C. during 18 hours in a self-regulating drying oven. The dried material so obtained had a dark brown color and weighed approximately 500 grams.

The dried material was then reduced and stabilized as follows. Approximately 300 grams of the material was placed in a glass tube heated in a horizontal furnace. A mixture of 2 volumes of nitrogen and 1 volume of hydrogen was passed over the catalyst at a temperature of 170 to 180° C. during 48 hours after which the reduction was complete as evidenced by the fact that water was no longer present in the effluent gases. The mixture of nitrogen and hydrogen was then displaced by nitrogen and thereafter a mixture of 60% nitrogen and 40% air was passed over the reduced material at room temperature for approximately 12 hours. The resultant material which was black in color was a stabilized active catalyst.

70 grams of benzoic acid, 63 grams of ethyl alcohol, and 15 grams of the above-described reduced and stabilized copper-alumina catalyst were placed in a rotatable steel autoclave, hydrogen was added to 100 atmospheres initial pressure, and the resultant reaction mixture was heated and rotated at 300° C. for a period of 4 hours. After this treatment, the autoclave and contents were cooled to room temperature and the reaction product was removed and analyzed. The reaction product consisted of toluene and ethyl benzoate in the respective yields of 39% and 30% of the theoretical based upon the benzoic acid charged.

*Example II*

70 grams of benzoic acid and 15 grams of the reduced and stabilized copper-alumina catalyst described in Example I were placed in a steel autoclave to which hydrogen was added to 100 atmospheres initial pressure, and the reaction mixture was then heated to 300° C. for four hours. The reaction product contained toluene in a yield of 41% of the theoretical together with small amounts of benzyl benzoate, benzaldehyde, and benzyl alcohol. Since the benzyl benzoate, benzaldehyde, and benzyl alcohol are apparently intermediates in the formation of toluene from benzoic acid, it is believed that the yield of toluene would have been increased appreciably by increasing the time of treatment with hydrogen at the reaction temperature.

The results of this example show that the hydrogenation is selective and does not involve the hydrogenation of the benzene ring of benzoic acid under the conditions of operation employed.

*Example III*

80 grams of phthalic anhydride and 15 grams of the reduced and stabilized copper-alumina catalyst described in Example I were placed in a steel autoclave of 850 cc. capacity under an initial hydrogen pressure of 150 atmospheres and heated to 300° C. for five hours. The 79.6 grams of recovered liquid product contained 8 grams of water. The liquid product was dried and was then separated by fractional distillation into the following fractions having the properties indicated.

| Fraction No. | Boiling point, °C. | Percent by volume | Refractive index $n_{D}^{20}$ |
|--------------|--------------------|-------------------|-------------------------------|
| 1.           | 102-114°           | 15.5              | 1.4955                        |
| 2.           | 114-120°           | 18.1              | 1.4973                        |
| 3.           | 120-141°           | 14.5              | 1.5002                        |
| 4.           | 141-147°           | 36.4              | 1.5048                        |
| 5.           | Residue            | 15.5              |                               |
|              | Total              | 100.0             |                               |

The predominant reaction was the formation of orthoxylene although some toluene was also formed.

The foregoing specification and examples indicate the character and value of the present process, although it is not intended that either section should unduly limit the generally broad scope of the invention.

We claim as our invention:

- 10 1. A process for producing alkyl aryl compounds which comprises reacting hydrogen and a member selected from the group consisting of aryl carboxylic acids and anhydrides of aryl carboxylic acids under hydrogenating conditions in the presence of a catalyst produced by subjecting to reduction a composite comprising copper oxide and at least another oxide selected from the group consisting of aluminum oxide and zinc oxide.
- 15 2. A process for producing alkyl aryl compounds which comprises reacting hydrogen and an aryl carboxylic acid under hydrogenating conditions in the presence of a catalyst produced by subjecting to reduction a composite comprising copper oxide and at least another oxide selected from the group consisting of aluminum oxide and zinc oxide.
- 20 3. A process for producing alkyl aryl compounds which comprises reacting hydrogen and an anhydride of an aryl carboxylic acid under hydrogenating conditions in the presence of a catalyst produced by subjecting to reduction a composite comprising essentially copper oxide and at least another oxide selected from the group consisting of aluminum oxide and zinc oxide.
- 25 4. A process for producing an alkyl aromatic hydrocarbon which comprises hydrogenating an aryl carboxylic acid in the presence of a catalyst produced by subjecting to reduction a composite comprising essentially copper oxide and at least another oxide selected from the group consisting of aluminum oxide and zinc oxide.
- 30 5. A process for producing an alkyl aromatic hydrocarbon which comprises reacting an aryl carboxylic acid and hydrogen at a temperature of from about 200° to about 350° C. in the presence of a catalyst produced by subjecting to reduction a composite comprising essentially copper oxide and at least another oxide selected from the group consisting of aluminum oxide and zinc oxide.
- 35 6. A process for producing an alkyl aromatic hydrocarbon which comprises reacting an aryl carboxylic acid and hydrogen at a temperature of from about 200° to about 350° C. under a pressure of from about 25 to about 300 atmospheres in the presence of a catalyst produced by subjecting to reduction a composite comprising essentially copper oxide and at least another oxide selected from the group consisting of aluminum oxide and zinc oxide.
- 40 7. A process for producing an alkyl aromatic hydrocarbon which comprises reacting an aryl carboxylic acid and hydrogen at a temperature of from about 200° to about 350° C. under a pressure of from about 25 to about 300 atmospheres in the presence of a catalyst produced by subjecting to reduction a composite comprising essentially a major proportion by weight of copper oxide and a relatively minor proportion of at least another oxide selected from the group consisting of aluminum oxide and zinc oxide.
- 45 8. A process for producing an alkyl aromatic hydrocarbon which comprises reacting an aryl carboxylic acid and hydrogen at a temperature of from about 200° to about 350° C. under a pressure of from about 25 to about 300 atmospheres in the presence of a catalyst produced by subjecting to reduction a composite comprising essentially a major proportion by weight of copper oxide and a relatively minor proportion of at least another oxide selected from the group consisting of aluminum oxide and zinc oxide.
- 50 9. A process for producing an alkyl aromatic hydrocarbon which comprises reacting an aryl carboxylic acid and hydrogen at a temperature of from about 200° to about 350° C. under a pressure of from about 25 to about 300 atmospheres in the presence of a catalyst produced by subjecting to reduction a composite comprising essentially a major proportion by weight of copper oxide and a relatively minor proportion of at least another oxide selected from the group consisting of aluminum oxide and zinc oxide.
- 55 10. A process for producing an alkyl aromatic hydrocarbon which comprises reacting an aryl carboxylic acid and hydrogen at a temperature of from about 200° to about 350° C. under a pressure of from about 25 to about 300 atmospheres in the presence of a catalyst produced by subjecting to reduction a composite comprising essentially a major proportion by weight of copper oxide and a relatively minor proportion of at least another oxide selected from the group consisting of aluminum oxide and zinc oxide.
- 60 11. A process for producing an alkyl aromatic hydrocarbon which comprises reacting an aryl carboxylic acid and hydrogen at a temperature of from about 200° to about 350° C. under a pressure of from about 25 to about 300 atmospheres in the presence of a catalyst produced by subjecting to reduction a composite comprising essentially a major proportion by weight of copper oxide and a relatively minor proportion of at least another oxide selected from the group consisting of aluminum oxide and zinc oxide.
- 65 12. A process for producing an alkyl aromatic hydrocarbon which comprises reacting an aryl carboxylic acid and hydrogen at a temperature of from about 200° to about 350° C. under a pressure of from about 25 to about 300 atmospheres in the presence of a catalyst produced by subjecting to reduction a composite comprising essentially a major proportion by weight of copper oxide and a relatively minor proportion of at least another oxide selected from the group consisting of aluminum oxide and zinc oxide.
- 70 13. A process for producing an alkyl aromatic hydrocarbon which comprises reacting an aryl carboxylic acid and hydrogen at a temperature of from about 200° to about 350° C. under a pressure of from about 25 to about 300 atmospheres in the presence of a catalyst produced by subjecting to reduction a composite comprising essentially a major proportion by weight of copper oxide and a relatively minor proportion of at least another oxide selected from the group consisting of aluminum oxide and zinc oxide.
- 75 14. A process for producing an alkyl aromatic hydrocarbon which comprises reacting an aryl carboxylic acid and hydrogen at a temperature of from about 200° to about 350° C. under a pressure of from about 25 to about 300 atmospheres in the presence of a catalyst produced by subjecting to reduction a composite comprising essentially a major proportion by weight of copper oxide and a relatively minor proportion of at least another oxide selected from the group consisting of aluminum oxide and zinc oxide.

of from about 200° to about 350° C. under a pressure of from about 25 to about 300 atmospheres in the presence of a catalyst produced by subjecting to reduction a composite comprising essentially copper oxide and aluminum oxide.

9. A process for producing an alkyl aromatic hydrocarbon which comprises reacting an aryl carboxylic acid and hydrogen at a temperature of from about 200° to about 350° C. under a pressure of from about 25 to about 300 atmospheres in the presence of a catalyst produced by subjecting to reduction a composite comprising es-

sentially copper oxide, zinc oxide, and aluminum oxide.

10. A process for producing an alkyl aromatic hydrocarbon which comprises reacting an aryl carboxylic acid and hydrogen at a temperature of from about 200° to about 350° C. under a pressure of from about 25 to about 300 atmospheres in the presence of a catalyst produced by subjecting to reduction a composite comprising essentially copper oxide and zinc oxide.

VLADIMIR N. IPATIEFF.  
VLADIMIR HAENSEL.